

## UNITED STATES PATENT OFFICE

2,614,982

METHOD OF PREVENTION OF CORROSION  
IN WELLS

Joseph A. Caldwell and Melba L. Lytle, Houston,  
Tex., assignors, by mesne assignments, to  
Standard Oil Development Company, Elizabeth,  
N. J., a corporation of Delaware

No Drawing. Application April 3, 1950,  
Serial No. 153,769

8 Claims. (Cl. 252—8.55)

1

This invention relates to a method of inhibiting the corrosiveness to corrodible ferrous metal surfaces of corrosive fluids containing hydrogen sulfide. More particularly, the invention relates to means for inhibiting the corrosivity of sulfide-containing, subsurface formation fluids to the corrodible conduits and attendant equipment through which the fluids are flowed and processed.

Crude oil containing soluble sulfides is often produced from subsurface formations and corrosion of conduits and attendant equipment is especially severe in those instances in which brine is produced along with the sour crude. Corrosive sulfide brines may include alkali metal sulfides, alkaline earth metal sulfides, acid sulfides such as hydrogen sulfide, and/or organic sulfides. Those brines containing hydrogen sulfide are especially corrosive to iron and steel equipment, the sulfides attacking the metal to form iron sulfide. Since these corrosive substances occur in or are introduced into the fluids originating in the subsurface formations, corrosion may occur throughout the conduits and attendant equipment through which the fluids from the subsurface formations are flowed and produced. In other cases the corrosion may be more or less localized to a limited portion of the conduits through which the fluids from the subsurface formations are produced. In any case, corrosion of the conduits and/or attendant equipment may be so severe as to require replacement of either or of both. Such replacements can be, and often are, extremely expensive. The expense involved is not limited merely to the cost of replacing the corroded equipment but may also involve killing the well in order to make repairs and to replace the corroded equipment. Not only is the cost of killing the well high but there is a marked loss in revenues due to having a well off production and to the necessity of having to maintain additional wells and sources of supply to meet production requirements during the period when the well is off production for repairs as a result of the corrosion. Corrosion may, on occasion, be so severe as to result in failure of the equipment in which event the well may flow wild. Enormous losses are incurred in such an eventuality.

The main object of the present invention is

5 to provide a method of substantially eliminating or inhibiting the corrosive action of subsurface fluids containing sulfides to conduits and attendant equipment through which the fluids are produced from the subsurface formations in which they originate.

In accordance with the present invention, corrosion of ferrous metal surfaces is inhibited or substantially eliminated by adding to fluid mixtures produced from subsurface formations and containing sulfides a small amount of fatty derivatives of polyethylene glycols. The lower molecular weight polyethylene glycols do not yield fatty derivatives which have practical effectiveness in inhibiting corrosion of ferrous metal surfaces by well fluids containing sulfides. For example, the fatty derivatives of mono-, di-, tri-ethylene glycols are either completely ineffective or must be used in prohibitive quantities to effect substantial inhibition. The most generally suitable and powerful fatty derivatives of polyethylene glycols are derived from polyethylene glycols of the type formula



25 in which C designates carbon, H designates hydrogen, O designates oxygen, and X has a value of from 3 to 30. It is preferred to employ a polyethylene glycol in which the value of X in the foregoing formula is in the range of 6 to 15. The  $(OC_2H_4)$  group in the foregoing formula will hereinafter be designated, for the sake of simplicity, as an ethoxy group. Fatty derivatives prepared from nonaethylene glycol, for example, are particularly effective. Other polyethylene glycols which may be mentioned by way of example include: tetraethylene glycol, pentaethylene glycol, hexaethylene glycol, heptaethylene glycol, octaethylene glycol, decaethylene glycol, dodecaethylene glycol, tridecaethylene glycol, pentadecaethylene glycol, etc.

30 The fatty material employed to produce the fatty derivatives of polyethylene glycol may be selected from the class of fatty acids and fatty oils. Acids having from 12 to 26 carbon atoms per molecule such as palmitoleic, oleic, ricinoleic, linoleic, linolenic, licanic, arachidonic, clupanodonic, lauric, myristic, arachidic, stearic, palmitic, etc. and fatty oils from which such acids can be 35 derived may be reacted with the polyethylene

glycols to produce the desired corrosion inhibiting agents. Especially effective agents are obtained by reacting the polyethylene glycols with such fatty oils as linseed oil, cottonseed oil, tung oil, oiticica, oil, China-wood oil, menhaden oil, and the like, or mixtures thereof. Likewise, mixtures of polyethylene glycols may be employed. In any event, the fatty material selected is reacted with the polyethylene glycol selected at a temperature in the range of from 300° to 550° F. for a time in the range of from 1 to 5 hours in the presence of a small amount of an alkaline reacting catalyst such as an alkali hydroxide or carbonate or mixtures thereof. The fatty derivatives of polyethylene glycols prepared in the foregoing manner are soluble in many aromatic solvents and, to a more limited extent, in petroleum solvents such as heavy naphtha or kerosene.

The polyethylene glycols which are employed in the preparation of the fatty derivatives of the present invention are readily available. They may be made, for example, by reacting ethylene oxide with water, the formation of polyethylene glycols being favored by maintaining the molal ratio of ethylene oxide to water in excess of 1. The degree of polymerization is determined by the reaction conditions maintained. Polyethylene glycols having molecular weights in excess of 1500 are commercially available as well as polyethylene glycols having lower molecular weights. For use in the preparation of the fatty derivatives employed in accordance with the present invention, it is not necessary that the polyethylene glycols be separated into close fractions of narrow molecular weight limits; on the contrary, fractions including a large number of polymers of different molecular weights may be employed.

When fatty derivatives of the present invention are prepared from a fatty oil and polyethylene glycol, it is preferable that the fatty oil be present in the initial reaction mixture in a weight ratio of from about 1:1 to about 3:1 as compared to the polyethylene glycol. When the fatty derivative is prepared from a fatty acid, the fatty acid should be present in the initial reaction mixture in a weight ratio of from about 0.5:1 to about 2:1 as compared to the polyethylene glycol. Only a small amount of the alkaline reacting catalyst need be present, and ordinarily no more than 3 weight per cent of the catalyst based on the weight of the reaction mixture is employed. For example, a concentration of 1 weight per cent of sodium hydroxide based on the weight of the reactants has been found sufficient to promote the reaction. On the other hand, as little as 0.5 weight per cent of sodium hydroxide based upon the weight of the reactants has been found sufficient when from about 0.5 weight per cent to about 2.0 weight per cent of sodium carbonate is utilized as a co-catalyst. In another instance 0.05 weight per cent of sodium hydroxide gave good results.

The amount of fatty derivative of the present invention employed to inhibit the corrosion of ferrous metal surfaces by well fluid mixtures containing hydrogen sulfide may be varied over a relatively wide range although it has been found that amounts within the range of 0.005 per cent to 0.1 per cent by volume of the fluid mixture give satisfactory results. Ordinarily, however, an amount within the range of 0.005 per cent to 0.01 per cent will give satisfactory inhibition.

Inasmuch as the fatty derivative of the present invention is soluble in certain solvents heretofore

mentioned, it may be found convenient to dissolve the fatty derivative in a suitable solvent before introducing it into the corrosive fluid mixture. When it is desired to protect from corrosion the conduit in the borehole, the fatty derivative or a solution thereof may be injected into the borehole adjacent the subsurface formation from which the corrosive fluid, including hydrogen sulfide, is produced or it may be introduced directly into the conduit through which the corrosive fluid flows from the subsurface formation to the surface of the earth. A still further method of introducing the fatty derivative into the fluids produced from the subsurface formation involves introducing the fatty derivative or a solution thereof into the annular space between the casing and the tubing. Another method of introducing the fatty derivative into the subsurface fluid consists of injecting the fatty material or a solution thereof into the subsurface reservoir through an adjacent well. Irrespective of the particular procedure employed in introducing the fatty derivative into the fluids in the well, the fatty derivative suppresses the corrosivity of the fluid, thereby eliminating or reducing damage to the conduit through which the fluids are produced and to attendant equipment through which the fluid is flowed.

In order to illustrate further the beneficial effects of the present invention, the following examples are given:

*Example I.*

Mild carbon steel coupons were immersed 31 times per minute for 14 days in a mixture containing 50 cc. of West Texas brine and 50 cc. of West Texas crude, the mixture being saturated with hydrogen sulfide. Air was excluded from the mixture. No inhibitor was added to this first mixture and it was employed as a control. Another mild carbon steel coupon was immersed 31 times per minute for 14 days in a mixture identical with the first mixture except that .01 per cent by volume of the reaction product of tung oil and nonaethylene glycol was added. A third carbon steel coupon was immersed 31 times per minute for 14 days in a mixture identical with the first mixture except that 0.005 per cent by volume of the reaction product of tung oil and nonaethylene glycol was added. This reaction product was prepared as follows: 60 grams of Chinese tung oil, 40 grams of nonaethylene glycol, and 0.5 gram of sodium hydroxide were heated together at a temperature of from 500° F. to 550° F. for a period of 2 hours. On completion of the reaction period, the reaction mixture was cooled to room temperature. The results obtained in the aforementioned tests are shown in Table I:

TABLE I

| Concentration of Inhibitor in Corrosive Fluid, Percent | Percent Reduction in Corrosion Over Blank |
|--------------------------------------------------------|-------------------------------------------|
| 0.01                                                   | 98                                        |
| 0.005                                                  | 55                                        |

Because the aforementioned laboratory tests indicated the marked effectiveness of fatty derivatives of polyethylene glycol as an inhibitor of the corrosivity of well fluids containing hydrogen sulfide, the reaction product of Chinese tung oil and nonaethylene glycol prepared in the manner hereinbefore indicated was field tested. This

field test was carried out by suspending mild steel coupons in the flow lines of two different wells, each of which was located in a different field, each well producing fluids containing hydrogen sulfide. Each coupon was retained in the flow line prior to inspection for a period of at least one week, and one coupon was allowed to remain in the flow line for a period of approximately 26 weeks. During certain portions of the test period the reaction product of Chinese tung oil and nonaethylene glycol was injected into the well fluids through the annulus between the casing and the tubing. The results obtained are tabulated below in Table II:

TABLE II

| Well    | Water Production, Percent | Oil Production Bbls./Day | Rate of Inhibitor Injection, Qts./Day | Time of Exposure, Days | Rate of Metal Loss, In./Yr. |
|---------|---------------------------|--------------------------|---------------------------------------|------------------------|-----------------------------|
| #1----- | 85                        | 5                        | 0                                     | 28                     | 0.0018                      |
|         | 85                        | 5                        | 0                                     | 30                     | 0.0021                      |
|         | 85                        | 5                        | a,b 1 1/2                             | 11                     | 0.0006                      |
|         | 85                        | 5                        | 1                                     | 35                     | 0.0003                      |
|         | 50                        | 25                       | 0                                     | 31                     | 0.031                       |
|         | 50                        | 25                       | 0                                     | 29                     | 0.065                       |
| #2----- | 50                        | 25                       | 0                                     | 7                      | 0.022                       |
|         | 50                        | 25                       | 0                                     | 25                     | 0.032                       |
|         | 50                        | 25                       | 0                                     | 184                    | 0.012                       |
|         | 50                        | 25                       | c 1                                   | 20                     | 0.028                       |
|         | 50                        | 25                       | 1                                     | 29                     | 0.0069                      |
|         | 50                        | 25                       | 1                                     | 33                     | 0.0036                      |

\* Inhibitor consisted of 88% reaction product of nonaethylene glycol and Chinese tung oil and 12% xylene by weight.

<sup>b</sup> Injection started 15 days prior to installation of coupon.

<sup>c</sup> Injection started 8 days prior to installation of coupon.

As indicated by the data in Table II, the reaction product of Chinese tung oil and nonaethylene glycol, in every case in which it was used, effected a marked reduction in the corrosion of the mild steel coupons.

Data on the material failures in well #2 support the evidence of the effectiveness of inhibition. Prior to the time that any inhibitor was injected into this well, a string of new tubing coated inside and out with a baked-on plastic was installed in the well. It was necessary to pull this tubing four times within the next 66 days following its installation because of failure of one or more joints, either by complete penetration of the pipe or by failure in the threads.

When it became necessary to pull the aforementioned tubing for the fourth time, it was replaced by a string of new, uncoated pipe. This newly installed string of pipe had to be removed and partly replaced in less than 3 months because one joint had corroded through. This same well, prior to the use of an inhibitor therein, had a further history of failures due to corrosion. For example, uncoated tubing has at times failed in 4 weeks and pump working barrels have failed in 30 days. In contrast to this history of repeated failures of the tubing in the well due to corrosion, no tubing failures occurred over a period of approximately 5 months from the time the inhibitor made from Chinese tung oil and nonaethylene glycol was first injected. Thus by injection of the aforementioned inhibitor into well fluids from this well, a marked reduction in corrosion of ferrous metal surfaces was obtained.

It will be observed from the data presented above that the addition of a small amount of a fatty derivative of polyethylene glycol effects a marked reduction in the tendency of a corrosive fluid solution containing hydrogen sulfide to corrode ferrous metal.

The nature and objects of the present invention having been fully described and illustrated,

what we wish to claim as new and useful and to secure by Letters Patent is:

- 5 1. A method for reducing the corrosiveness to corrodible ferrous metal of a corrosive-petroliferous well fluid including moisture and hydrogen sulfide which comprises introducing into said fluid a corrosion inhibiting amount of a reaction product obtained by reacting a fatty material selected from the group consisting of fatty acids having at least 12 and no more than 26 carbon atoms per molecule and fatty oils containing fatty acid radicals having no less than 12 and no more than 26 carbon atoms in the radical with a polyethylene glycol containing at least 3 and no more than 30 ethanoxy groups at a temperature in the range of 300° to 550° F. for a period of from 1 to 5 hours in the presence of an alkaline reacting catalyst selected from the group consisting of alkali metal hydroxide and alkali metal carbonate, the weight ratio of fatty material to polyethylene glycol being in the range of 1:1 to about 3:1.
- 10 2. A method in accordance with claim 1 in which the reaction product is added to the corrosive fluid in an amount within the range of 0.005% to 0.1% by volume of the fluid.
- 15 3. A method for reducing the corrosiveness to corrodible ferrous metal of a corrosive-petroliferous well fluid including moisture and hydrogen sulfide which comprises introducing into said fluid a corrosion inhibiting amount of a reaction product formed by heating tung oil and nonaethylene glycol together for a period of from 1 to 5 hours at a temperature in the range of 300° to 35 550° F. in the presence of an alkaline reacting catalyst selected from the group consisting of alkali metal hydroxide and alkali metal carbonate, the weight ratio of tung oil to nonaethylene glycol being in the range of 1:1 to about 3:1.
- 40 4. A method in accordance with claim 3 in which the reaction product is added to the corrosive fluid in an amount within the range of 0.005% to 0.1% by volume of the fluid.
- 45 5. A method for reducing the corrosiveness to corrodible ferrous metal of a corrosive-petroliferous well fluid including moisture and hydrogen sulfide which comprises introducing into said fluid a corrosion inhibiting amount of a reaction product formed by heating cottonseed oil and nonaethylene glycol together for a period of from 1 to 5 hours at a temperature in the range of 300° to 550° F. in the presence of an alkaline reaction catalyst selected from the group consisting of alkali metal hydroxide and alkali metal carbonate, the weight ratio of cottonseed oil to nonaethylene glycol being in the range of 1:1 to about 3:1.
- 50 6. A method in accordance with claim 5 in which the reaction product is added to the corrosive fluid in an amount within the range of 0.005% to 0.1% by volume of the fluid.
- 55 7. A method for reducing the corrosiveness to corrodible ferrous metal of a corrosive-petroliferous well fluid including moisture and hydrogen sulfide which comprises introducing into said fluid a corrosion inhibiting amount of a reaction product formed by heating oiticica oil and nonaethylene glycol together for a period of from 1 to 5 hours at a temperature in the range of 300° to 550° F. in the presence of an alkaline reaction catalyst selected from the group consisting of alkali metal hydroxide and alkali metal carbonate, the weight ratio of oiticica oil and nona-
- 60
- 65
- 70
- 75

ethylene glycol being in the range of 1:1 to about 3:1.

8. A method in accordance with claim 7 in which the reaction product is added to the corrosive fluid in an amount within the range of 0.005% to 0.1% by volume of the fluid. 5

JOSEPH A. CALDWELL.  
MELBA L. LYTHE.

## REFERENCES CITED

The following references are of record in the file of this patent:

## UNITED STATES PATENTS

| Number    | Name   | Date          |
|-----------|--------|---------------|
| 2,249,800 | Weber  | July 22, 1941 |
| 2,460,259 | Kahler | Jan. 25, 1949 |
| 2,527,889 | Moore  | Oct. 31, 1950 |

## OTHER REFERENCES

Ind. & Eng. Chem., vol. 40, No. 12, page 2344.  
Article by Baker et al.